

# United States Patent

[19]

Amend

[11] 3,883,302

[45] May 13, 1975

[54] HIGH-BULK POLYACRYLONITRILE YARN

[75] Inventor: Werner Amend, Wuppertal-Barmen, Germany

[73] Assignee: Hacoba-Textilmaschinen GmbH & Co. KG, Wuppertal-Barmen, Germany

[22] Filed: Dec. 26, 1972

[21] Appl. No.: 318,560

## Related U.S. Application Data

[63] Continuation of Ser. No. 90,034, Nov. 16, 1970, abandoned.

[52] U.S. Cl. .... 8/172; 8/93; 8/173; 8/175; 8/177 R

[51] Int. Cl. .... D06p 5/06

[58] Field of Search .... 8/93, 172, 175, 177 AB, 8/177 R, 173

## [56] References Cited

### UNITED STATES PATENTS

|           |         |                    |          |
|-----------|---------|--------------------|----------|
| 2,404,718 | 7/1946  | Houtz .....        | 260/30.8 |
| 2,953,420 | 9/1960  | Hees et al. ....   | 8/172    |
| 3,051,736 | 8/1962  | Ham .....          | 8/177    |
| 3,114,588 | 12/1963 | Lewis .....        | 8/177    |
| 3,116,103 | 12/1963 | Gamlen et al. .... | 8/18     |

|           |        |               |       |
|-----------|--------|---------------|-------|
| 3,117,831 | 1/1964 | Mautner ..... | 8/175 |
| 3,529,927 | 9/1970 | Ulrick .....  | 8/173 |
| 3,558,260 | 1/1971 | Hermes .....  | 8/21  |

## FOREIGN PATENTS OR APPLICATIONS

891,907 3/1962 United Kingdom..... 8/177

## OTHER PUBLICATIONS

Ham, Ind. & Eng. Chem., Vol. 46, No. 1, pp. 390-392.

Neary et al., Amer. Dyestuff Reporter, Vol. 46, No. 17, pp. 625-633.

Primary Examiner—Benjamin R. Padgett

Assistant Examiner—Peter A. Nelson

Attorney, Agent, or Firm—Karl F. Ross; Herbert Dubno

## [57] ABSTRACT

Dyed, highly-bulked yarns of polyacrylonitrile fibers are produced by treating the yarns below their melting point with an acid liquor which in addition to a cationic dye also contains a compound which swells and/or starts dissolving the fibers. After this treatment, the yarns are subjected to a damp heat treatment at temperatures of at least 98° preferably in the range from 98° to 100°.

1 Claim, No Drawings

**HIGH-BULK POLYACRYLONITRILE YARN**

This is a continuation of application Ser. No. 90,034, filed Nov. 16, 1970, now abandoned.

**FIELD OF INVENTION**

The invention relates to high-bulk polyacrylonitrile yarn and a method of making same.

**BACKGROUND OF THE INVENTION**

It is known to dye and bulk polyacrylonitrile yarns which consist of mixtures of shrinkable and non-shrinking fibers. Cationic dyes in acid media are used as the coloring substances. There are two usual methods for the manufacture of dyed and bulked yarns.

In the first method, the non-bulked yarns brought from the spinning mill to the cops are first made into larger coils (crosscoils, bobbins) and are then reeled into strands, after which they are dyed for 2 to 4 hours in a suspending apparatus, using a liquor ratio in the range from 1:30 to 1:60 at a temperature in the range of 75° to 106°C, whereby either the dye bath must be slowly heated (at about 0.5°C per minute) from 75° to 100°C, or in a low-pressure apparatus to 106°C or, in the case of a temperature in the range from 80° to 100°C, this must be maintained for 45 to 90 minutes and then left at 100°C or 106°C for at least 15 minutes.

It is a feature of both of these variations of the method that the yarn must be heated to 100°C or 106°C for a specific time so that the shrinkable portion of the yarn can shrink and the bulking effect can thus be achieved. After heating to 100° or 106°C, in both these variations, the liquor must be slowly cooled (about 1°C per minute) so that the bulking effect and feel of the fabric are retained. After the usual secondary treatment, the strands must then be converted into coil form for subsequent use, e.g. for knitting.

Apart from the fact that this method is uneconomical due to the high liquor ratio, the expensive reeling of coiled shapes into strands and the particularly expensive rewinding of strands into coils, it also has the disadvantage that the yarn is distorted by the movement of the liquor and that the positions of the strands on the bars of the dyeing machine become clearly marked.

In the second method, the yarns from the spinning mill on the cops are wound into a special form, namely such that a coiled body is obtained which enables the yarns to be shrunk during the dyeing process at 75° to 106°C without a solid casing. Apart from the fact that special and unusual winding apparatus is required, this method also has the disadvantage that the cross-over points of the threads are clearly marked. This method is therefore only used in practice for simple (i.e. un-twisted) and fine yarns. The second variation of the first method is also possible with this method. For subsequent treatment, the yarns must generally be wound on to the user spools.

In both methods, it is impossible to dye the yarns below the melting point of the threads (in technical terms, the "glass transformation point" or glass transition temperature—see pg. 116-117 of WHITTINGTON'S DICTIONARY OF PLASTICS, First Edition, Technomic Pub. Co., 1968), which generally lies at about 80°C in fibers which are usually dry-spun and about 70°C in fibers which are usually wet-spun.

It is furthermore already known to dye and bulk knitted articles, e.g. pullovers or sleeves, of polyacrylonitrile yarns, in which the yarn consists of a mixture of

shrinkable and non-shrinking fibers, with cationic dyes, by treating them for 2 to 4 hours with an acid liquor which contains the dissolved cationic dye, at a temperature in the range from 75° to 100°C, whereby either 5 the liquor is slowly heated (about 0.5° per minute) or in the case of a temperature in the range of 80° to 95°C, this is maintained for 45 to 90 minutes and the bath is then heated to 100°C and is retained at this temperature for at least 15 minutes. The treatment of the 10 shaped articles takes place in paddle-dyeing machines, but in order to avoid distortion, the articles must be sewn into pouches. In order to overcome this difficulty, the shaped articles are treated on specially developed apparatus which does not have paddles but uses nozzles 15 to move the liquor.

For smooth finishing, after treatment with the dyeing liquor and the usual rinsing, finishing and drying steps, the shaped articles are wound onto formers and are steamed at 98° to 100°C. Since yarn shrinkage of up to 20 about 25% occurs in the shaped articles in the event of treatment with the hot to boiling dyeing liquor visible different final dimensions of the shaped articles often result. Moreover, strong warping of the shaped articles 25 cannot be avoided and unusable merchandise is obtained.

It is also known to dye and bulk flat sheet-like textile material of polyacrylonitrile yarns which consist wholly or partially of a mixture of shrinkable and non-shrinking polyacrylonitrile fibers in acid baths with cationic dyes, whereby the treatment of the textile material takes place for example on a jigger, beam dyeing machine, winch machine or star-frame dyeing machine 30 and the processing liquors likewise have temperatures above the glass transformation point. In this method, 35 the flat sheet-like textile material contracts so much that a satisfactorily uniform dye penetration of the yarn is not possible. Furthermore, distortions and warping occur through the practically uncontrollable shrinkage and the mechanical stresses. Also the feel of the fabric is impaired by the distortion of the yarn; a flattened yarn which is crushed at the cross-over points is obtained.

**OBJECT OF THE INVENTION**

45 It is the object of the invention to provide an improved high-bulk dyed polyacrylonitrile yarn and a method of making same.

**SUMMARY OF THE INVENTION**

50 It has now been found that dyed, highly-bulked yarns of polyacrylonitrile fibers can be produced by treating the yarns below their melting point with an acid liquor which, in addition to a cationic dye, also contains a compound which swells and/or starts dissolving the fibers and, after the treatment, subjecting the yarns to a damp heat treatment at temperatures of at least 98°, 55 preferably in the range of 98° to 100°C.

**SPECIFIC DESCRIPTION**

60 With the method of the invention, the temperature of the dyeing liquor always lies beneath the glass transformation point of the fibers and generally amounts to 40°C to 79°C, preferably 60°C to 75°C, whereby the lower temperatures are preferably chosen for wet-spun fibers and the higher temperatures for dry-spun fibers. The processing time with the dyeing bath amounts to 65 10 to 90 minutes, preferably 30 to 60 minutes.

The cationic dyes used are sufficiently known, as are the usual liquor additives, such as acetic acid which are used for coloring the polyacrylonitrile yarns.

After the treatment with the dyeing liquor, rinsing and finishing is carried out in the usual manner.

With the method according to the invention, yarns which are wound on to spools can be subjected to treatment with the acid dyeing liquor and then rinsed, finished, centrifuged or drawn off in the usual way. Thereafter, the wound damp yarns are rewound onto the user spools, which is necessary for subsequent treatment whereby during the rewinding process, the yarns are subjected while free of tension to the damp-heat treatment. They thereby pass through a zone in which they are heated, preferably at temperatures in the range of 98° to 100°C. In this heating zone, the necessary temperature can be produced for example by means of steam, infrared rays, microwaves or hot air. The length of heating depends on the residual moisture of the yarns and on the amount of dye applied. The heating times are from 2 to 15 minutes, preferably from 4 to 10 minutes, but heating times of 5 to 20 seconds may also produce a useful effect. The rate of flow depends on the size of the heating zone. The yarn preferably leaves the heating zone in the dry state. In order to guarantee a bulking effect, the yarn must be passed, free of tension, through the heating zone according to one of the conventional methods, e.g. by way of a wire cloth or by cuttling in a chamber-like heating zone.

According to a further feature of the invention, the yarns are first processed into shaped articles and then subjected to treatment with the acid dyeing bath and afterwards place on molds or formers for the heat treatment. The shaped articles are thus placed on the molds after finishing and possibly centrifuging and are then steamed, whereby the shaped articles are shrunk to the desired shape.

Moreover, the yarns to be treated according to the invention can also be subjected to the dyeing process in the form of flat sheet-like material, e.g. as fabric, knitted texture, knitting or sections of tubular fabrics or circular knitted goods. In this form, these textile materials are steamed for 10 seconds to 10 minutes, preferably from 30 seconds to 5 minutes. Steaming is carried out on the usual steaming apparatus, such as a screen belt or perforated drum steamer, or a steam-coated tenter frame, and can be so arranged that specific final dimensions of the textile fabric are obtained.

The compounds required for the method according to the invention to swell and/or start to dissolve the fibers in an aqueous medium are already partly known as such from technical literature, but can however easily and quickly be discovered by the expert. In order to find out, a yarn sample of about 10 g need only be treated in 200 cc of a liquor for 45 minutes at 65°C, wherein the liquor contains, per liter of water, 1 cc of 60% acetic acid, 0.5 g of the yarn dye material including Color Index No. 48055

in the usual form and condition and 60 g of the substance to be tested. As opposed to a control sample (without a swelling or solvent substance), the yarn must be dyed twice as deep. It is clear to the expert that

5 with this test a large number of substances can be tested next to one another at the same time, whereby in addition the minimum amount of material required can be ascertained. If solid products which are insoluble in water are to be tested, they are first dissolved in 10 an organic solvent chosen such that an excess of solvent is not harmful; with aliphatic compounds, in e.g. polyglycols, with aromatic compounds, generally in benzyl alcohol to which methanol is added in the same amount as the benzyl alcohol and about 10% by weight of a conventional nonionic emulsifier is added to these 15 solutions. A general addition of methanol in a ratio of 1:1 and of a nonionic commercial emulsifier in the ratio of 1:0.1 is preferable however, particularly when the 20 tester does not first want to check the exact solubility of the products in the usual technical books. In the case of liquid compounds which are insoluble in water, a conventional nonionic emulsifier in the ratio 1:0.1 to 1:0.8 is added to the products, preferably with an alcohol such as methyl or ethyl alcohol in the ratio of 1:1.

25 As regards swelling or dissolving compounds, the following 52 in are preferred:

30 Diesters of carbonic acid, especially cyclic diesters of carbonic acid with glycols, in particular with ethylene and propylene glycols, whose carbonic diesters are referred to technically as ethylene or propylene carbonate, aliphatic, cycloaliphatic and aromatic mono-and 35 dinitriles, which if required can be substituted and moreover, can contain heteroatoms, such as for example oxygen and nitrogen, between two carbon atoms; by way of example, acetonitrile, propionitrile, benzyl oxypropionitrile



phenylacetonitrile, benzonitrile, succinonitrile, azelaic dinitrile and phthalonitrile.

45 Mononitriles substituted with a phenyl group are preferably used. Benzyl oxypropionitrile is particularly suitable as regards efficiency and possible toxicity.

50 It is obvious that mixtures of these compounds may also be used. As a rule, a solution must first be prepared from those compounds which are solid and insoluble in water and an emulsifier is then added to the solution. With aliphatic compounds, an aliphatic monohydric or polyhydroc alcohol, e.g. methanol, ethanol or glycol, is 55 preferably used as the solvent and, with aromatic compounds, benzyl alcohol is preferably used, to which methanol is added after the dissolving process in the ratio of benzyl alcohol to methanol of 1:4 to 4:1 parts by weight. Only nonionic products, particularly the ethoxylated products of alkylphenols, and moreover the 60 ethoxylated products of fatty acid esters, fatty alcohols and fatty amines and the alkylpolypropylene glycol-polyglycol ethers, are suitable as emulsifiers. Furthermore, polyalkylene oxides, e.g. polyglycols or mixed 65 products of unsubstituted polypropylene oxide and polyethylene oxide units are suitable as emulsifiers, for, at least, the emulsifying effect of nonionic emulsifiers is clearly improved by the addition of such compounds.

(A)



Water-soluble substances, e.g. ethylene and propylene carbonates, can be added to the dye bath without any other additives. An emulsifier is preferably added to liquid compounds, which are insoluble in water, in a ratio of 5:1, though a higher amount does not have a disadvantageous effect. Also, an addition of alcohol has a particularly favorable effect. For economical reasons, the additive should normally not be higher than 1:1, 3 to 60 g and, generally, 5 to 40 g per liter of the compounds which swell and/or dissolve the fibers are added to the dye bath. The amount to be added depends on the amount of dye used, the dye temperature and the type of fiber; higher amounts of dye, lower temperatures and dry-spun fibers require higher quantities and vice versa.

As contrasted with the most common method, namely treatment in strand form with yarns of the instant invention the expensive unwinding and the even more subsequent rewinding of the strands are dispensed with. The spool losses are much less with the method according to the invention and the kink-free lengths are longer. Moreover, high liquor ratios are avoided. As distinct from the treatment on special spools, with the method according to the invention, only the normal winding machines are required and, furthermore, twisted and coarse yarns may also be treated. As opposed to all the known methods, there is in addition the great advantage that no marking spots occur and the swelling effect is more favorable since a voluminous yarn results.

Passing the yarn through the heating zone does not represent an additional working step for even with the known method, drying and rewinding also take place.

If the yarns are in the form of shaped articles, the method according to the invention has the advantage over the known methods in that no special dyeing machines are required, but processing can take place in the paddle machine without the articles having to be sewn into sacks, since distortion and warping do not occur.

If the yarns are in the form of flat, sheet-like textile material, the method according to the invention has the advantage that the yarns do not become flattened or crushed at the crossover points, and furthermore, that distortions and warping do not occur, but a very good dye penetration is obtained.

It is surprising that a method like that of the invention is possible; when dyeing polyacrylonitrile fibers with cationic coloring substances, in order to avoid any irregularities, long processing times with very long heating up times are required and special compounds, so-called retarders, are added with in addition retard the taking up of the coloring substances, while the method according to the invention succeeds using only short processing times, temperature stability and no retarders. However no irregularities occur. It is furthermore surprising that compounds which have a swelling and/or dissolving effect on the fibers in the method according to the invention have no adverse influence on the technological properties of the fibers, particularly the breaking tension. Furthermore, it is stated in technical literature that it is not possible to dye polyacrylonitrile fibers beneath the melting point of the fibers (glass transformation point). Thus the expert is considerably prejudiced against the practicability of a method of the type according to the invention.

## SPECIFIC EXAMPLES

## EXAMPLE 1

5 A 600 g cross-coiled spool of polyacrylonitrile yarn which consisted of shrinkable and non-shrinking wet-spun fibers and had a yarn thickness of Nm 22/2\*, was treated with a liquor in the ratio of 1:10 for 60 minutes at 65°C on a cross-coil machine, the liquor containing, in 1 liter of water, 1 g of dyestuff (A), Color Index No. 10 48055



20 in the usual form and quality, 1 cc of 60% acetic acid and 30 g propylene carbonate. \*The thickness measurement Nm 22/2 indicates a double twist (2) and a specific length of 22 meters per gram.

25 It was then hot and cold rinsed, finished and centrifuged. The yarn was then continuously cutted on an endless screen belt, treated with saturated steam at 100°C and then dried by means of hot air and wound on to a cone. A highly bulked, voluminous, dark yellow yarn without any markings or irregularities was obtained.

## EXAMPLE 2

30 Shaped articles weighing 10 kg and consisting of polyacrylonitrile yarns which comprises shrinkable and non-shrinking wet-spun polyacrylonitrile fibers were treated with liquor in a ratio of 1:50 for 60 minutes at 35 65°C in a paddle dyeing machine, the liquor containing in 1 liter of water 0.2 g of the following dye:



in the usual form and quality;

1 cc of 60% acetic acid,  
50 5 g benzyloxypropionitrile dissolved in  
0.4 g benzyl alcohol  
0.8 g methanol  
1.0 g of a polyglycol ester with 10 mol ethylene oxide  
0.8 g of an adduct of propylene oxide and ethylene  
oxide of average molecular weight 1500.

55 It was then hot and cold rinsed, finished and dried. The shaped articles were then placed on suitable formers and steamed for 4 minutes.

## EXAMPLE 3

60 A fabric of polyacrylonitrile yarn which consisted in the warp of Nm 80/2 non-shrinking polyacrylonitrile yarn and in the weft of Nm 60/2 polyacrylonitrile yarn with shrinking and non-shrinking fibers, woven in a width of 1.60 m, was treated on a jigger in a liquor ratio of 1:5 for 45 minutes at 65°C with a liquor which contained in 1 liter:

65 2 g of dyestuff, Color Index No. 48020



in the usual form and quality

1 cc of 60% acetic acid

8 g propionitrile

8 g methanol

0.8 g of a reaction product of ricinoleic acid with 36 mol ethylene oxide.

After the usual rinsing, finishing and drying, the fabric was passed through a steam-heated tenter frame with an adjoining hot-air compartment which was set to a final width of 1.25 m. The speed of the tenter frame was so adjusted that a steaming time of 2 minutes was reached and the cloth left the frame in a dry condition.

10

15

20

25

30

35

40

45

50

55

60

65

I claim:

1. A method of making high-bulk polyacrylonitrile yarn covered with cationic dyes, which comprises the steps of treating unbulked polyacrylonitrile yarn in a bath at a temperature beneath 70°C and its glass transition temperature with an aqueous acid liquor containing a cationic dye and benzyloxypropionitrile as a polar organic compound which swells or solubilizes the fibers of said yarn, and thereafter subjecting the yarn to damp heat treatment at a temperature of substantially 98°C to 100°C, the yarn being subjected to the treatment with the aqueous acid liquor while coiled on spools, is then rinsed, finished and centrifuged and is finally re-wound from the spools on to user spools while being maintained free from tension during the rewinding process during the damp heat treatment for a period of 5 seconds to 15 minutes.

\* \* \* \* \*